

Patented Aug. 21, 1928.

1,681,540

# UNITED STATES PATENT OFFICE.

OLIVER T. HUNGERFORD, OF BELLEVILLE, NEW JERSEY.

## PACKING MATERIAL.

No Drawing.

Application filed April 12, 1927. Serial No. 183,246.

My invention relates to a material designed primarily for use as a packing or for upholstering. It is particularly desirable for use as journal box packing and may be used for all kinds of upholstering where a light, resilient material is desired. The object is not only to provide a superior product for the purposes, but to obtain said product from material which has heretofore been considered largely a waste material and of no particular value. The product obtained possesses many advantages over others commonly used for the purposes indicated. First, it is much less expensive, it is more elastic and resilient as a packing or upholstering material, has greater absorbing capacity for oil and gives off the oil more freely when used for such purposes as journal box packing, and may be obtained in limited quantities at a comparatively small cost.

In manufacturing the product, I take the flax straw, which, as is well known, consists of a fibrous, gummy and woody substance, and subject the same to a chemical treatment as by boiling it in a bath of caustic soda or appropriate combination of sodas, to remove the gum and to facilitate the separation of the fiber from the woody portion or shive, which process is well known to those skilled in the art, and then dry the same, then pass it through a decorticating machine. The resulting product is a fine, fibrous, fluffy, wooly mass of great absorbing qualities. With this I mix an appropriate quantity of a harder, more resilient, material such as sisal fiber, which has an inherent resiliency and, when appropriately mixed with the flax fiber, lends to the mass an elasticity and resiliency which makes it peculiarly desirable for the purposes stated. Instead of the sisal fiber, a harder, tougher portion of the flax straw, or some other similar material may be substituted.

It will be understood, of course, that the proportion of this hard, resilient, woody fiber used will depend upon the purpose for which the resulting product is intended. Where cheap upholstery or packing is intended, more of the harder, tougher portion of the flax shive or cheaper substance can be employed. Where a higher class material is desired, a smaller proportion of the sisal fiber or other material and more of the flax fiber is employed.

In actual practice it has been found that the material constituting this invention is much lighter than other material commonly used for the same purpose, and that the same or better results can be secured by the use of a much smaller quantity by weight; that the cost per pound is likewise much less than the cost per pound of material commonly used for like purposes; that when used as a packing for journal boxes a much larger quantity of oil is taken up or absorbed or carried by the same quantity of the material of this invention than by a corresponding quantity of other materials commonly used for such purposes; further, the oil is given off to the journal more freely because of the more fluffy, porous and resilient character of the packing than is the case when packing of other materials is employed. When used for upholstery the material is found to retain its resilient character and does not "pack" and become hard as is the case with many other materials used for like purposes. All of these conditions tend to enhance the value of the invention and testify to its importance in the art.

It will be understood, of course, that various modifications in my invention may be made without departing therefrom, the substance of the invention consisting in providing a product consisting of flax fiber mixed with a harder, resilient substance to produce a product for the purposes stated.

Having thus fully described my invention, what I claim as new and desire to secure by Letters Patent is:

1. A packing material consisting of fibrous material recovered from flax straw and having mixed therewith a percentage of harder, flexible, resilient substance, substantially as set forth.

2. A packing material consisting of flax fiber recovered from flax straw by de-gumming said straw and mixing with said flax fiber a percentage of sisal fiber, substantially as set forth.

3. A packing material consisting of flax fiber mixed with a harder, tougher and more resilient substance, substantially as set forth.

In witness whereof, I have hereunto set my hand at Washington, District of Columbia, this 8th day of April, A. D. nineteen hundred and twenty-seven.

OLIVER T. HUNGERFORD.